

## UNITED STATES PATENT OFFICE

2,409,746

## MOTOR FUELS

Theodore W. Evans, Oakland, and Alfred G. Cattaneo, Berkeley, Calif., assignors to Shell Development Company, San Francisco, Calif., a corporation of Delaware

No Drawing. Application July 31, 1940,  
Serial No. 348,838

4 Claims. (Cl. 44—56)

1

This invention relates to motor fuels for use in high compression internal combustion spark ignition engines and relates more particularly to motor fuels blended with an agent which tends to reduce the knocking of the fuel in supercharged gasoline engines.

Branched chain ethers, such as di-isopropyl ether, have been suggested as blending agents to raise the octane rating of low octane fuels. Their primary value lies in their own high octane ratings, and by virtue of this property raise the octane rating of the hydrocarbons which are the primary source for motor fuels.

Low octane fuels have been considered the most susceptible to the beneficial action of the ethers. Blending with hydrocarbon fuels having octane ratings equal to or greater than those of the ether, however, was considered disadvantageous because no improvement in octane rating is effected, while the B. t. u. content of the blended fuel is reduced, it being well known that the B. t. u. values of the ethers are much below those of hydrocarbons.

We have now found that certain blends of ethers with hydrocarbons, which blends possess octane numbers not substantially greater than those of the hydrocarbons alone prove vastly superior to the straight hydrocarbons in supercharged engines. Such blends are obtained when mixing certain ethers with hydrocarbons having octane ratings equal to or higher than the particular ethers. Some few hydrocarbons of lower octane than the ethers produce blends which have still lower octane number than the hydrocarbons.

Certain asymmetrical dialkyl ethers, one alkyl group of which is a tertiary alkyl radical, preferably of 4 to 6 carbon atoms such as tertiary butyl radical, and the other alkyl group of which contains 1 to 3 carbon atoms in a straight or branched chain, have octane ratings of 100 or slightly lower. Blends thereof with hydrocarbon fuels of equal or higher octane number have octane ratings not higher than those of the hydrocarbon fuel alone, but peculiarly enough permit more efficient opera-

2

tion of supercharged spark ignition engines than the latter.

As is known, supercharging is one method of markedly raising the power output of gasoline engines. This method comprises boosting the intake pressures to above atmospheric pressure, thus increasing the compression pressures. The degree of supercharging is limited by the knocking property of the fuel, for all fuels have a critical compression pressure above which they detonate spontaneously. Obviously the fuel which permits the highest degree of supercharging is the most desirable.

Response to supercharging may be measured by a unit known as the "allowable boost ratio" or A. B. ratio which is determined as follows:

The intake pressure of an engine running at constant speed and constant compression ratio is measured when a certain arbitrary degree of knocking takes place. Thereafter the engine is run on a reference fuel at the same speed and compression ratios, with varied intake pressure until the same degree of knocking is obtained.

The intake pressure of the blended fuel divided by the intake pressure of the reference fuel gives the A. B. ratio of the blended fuel. By convention the A. B. ratio is based on iso-octane as the reference fuel.

Examples of ethers suitable for our invention are methyl tertiary butyl ether, methyl tertiary amyl ether, methyl tertiary hexyl ether, ethyl tertiary butyl ether, n-propyl tertiary butyl ether, isopropyl tertiary butyl ether, isopropyl tertiary amyl ether, etc.

The amounts of the ethers used in the blends are advantageously at least about 5% and preferably from 5% to 50%, although quantities outside these limits may be used if desired.

In the table below, examples of blends of hydrocarbons with the above ethers are shown, which blends have equal or lower octane ratings than the hydrocarbons, but possess materially increased A. B. ratios.

| Ether                       | Hydrocarbon                |                |                      | Blend                       |                      |                |
|-----------------------------|----------------------------|----------------|----------------------|-----------------------------|----------------------|----------------|
|                             | Name                       | A. B.<br>ratio | ASTM<br>oct. No.     | Percent<br>ether by<br>vol. | ASTM<br>oct. No.     | A. B.<br>ratio |
| Methyl tertiary butyl ether | Triptane                   | 1.35           | 1 101 <sup>3/4</sup> | 50                          | 1 101 <sup>3/4</sup> | 1.45           |
| Do.                         | 50% iso-octane, 50% xylene | 1.15           | 97                   | 33 <sup>1/2</sup>           | 96 <sup>1/2</sup>    | 1.30           |
| Do.                         | 80% iso-octane, 20% xylene | 1.10           | 100                  | 50                          | 99 <sup>1/2</sup>    | 1.30           |
| Methyl tertiary amyl ether  | Iso-octane                 | 1.0            |                      | 50                          | 99                   | 1.20           |

<sup>1</sup> Determined with the aid of iso-octane containing .05 cc. tetra ethyl lead.

It will be seen that the addition of various quantities of our ethers, while failing to improve the octane rating, markedly increases the allowable boosting of the intake pressure without causing knocking.

Suitable gasoline hydrocarbons with which to blend the ethers are, for example, iso-octane, neo-hexane, triptane, mixtures of polymer or alkylate gasoline with triptane, mixtures of iso-octane, neohexane, triptane, isopentane, etc., blends of relatively low boiling aromatic hydrocarbons such as toluene, xylenes, ethyl benzene, etc. with high octane aliphatic hydrocarbons, etc.

If desired, anti-detonants such as, tetraethyl lead, aniline, mono methyl aniline, or anti-oxidants such as phenols, aminophenols, may be added to our blended fuels.

We claim as our invention:

1. An improved motor fuel for supercharged spark ignition engines comprising a mixture of methyl, tertiary butyl ether and gasoline hydrocarbons containing a substantial amount of iso-octane, said mixture having an octane rating lower than said hydrocarbons, and said fuel having an A. B. ratio greater than that of said gasoline hydrocarbons.

25

2. An improved motor fuel for supercharged spark ignition engines comprising a mixture of methyl tertiary butyl ether and gasoline hydrocarbons containing a substantial amount of triptane, said mixture having an octane rating lower than said hydrocarbons, and said fuel having an A. B. ratio greater than that of said gasoline hydrocarbons.

3. An improved motor fuel for supercharged spark ignition engines comprising a mixture of methyl tertiary butyl ether and gasoline hydrocarbons containing a substantial amount of neohexane, said mixture having an octane rating lower than said hydrocarbons, and said fuel having an A. B. ratio greater than that of said gasoline hydrocarbons.

4. An improved motor fuel for supercharged spark ignition engines comprising a mixture of methyl tertiary butyl ether and gasoline hydrocarbons containing a substantial amount of hydrocarbons selected from the group consisting of iso-octane, neohexane, triptane, and mixtures thereof.

THEODORE W. EVANS.  
ALFRED G. CATTANEO.